

Oct. 12, 1948.

G. W. JERNSTEDT

2,451,341

ELECTROPLATING

Filed Aug. 10, 1945

Fig. 1.



Fig. 2.



Fig. 3.



Fig. 4.



Alternating Current Plating

Fig. 5.



WITNESSES:

Edward Michaels

J. Shapoe

Fig. 6.



INVENTOR

George W. Jernstedt.

BY

Era W. Savage

ATTORNEY

## UNITED STATES PATENT OFFICE

2,451,341

## ELECTROPLATING

George W. Jernstedt, Belleville, N. J., assignor to  
Westinghouse Electric Corporation, East Pitts-  
burgh, Pa., a corporation of Pennsylvania

Application August 10, 1945, Serial No. 610,107

10 Claims. (Cl. 204—44)

1

This invention relates to electroplating and, more particularly, to a novel process and the product produced thereby.

In applying to base members electrodeposits of metals, it is desirable to produce a predetermined thickness of electrodeposit as rapidly as possible with as high a quality as is reasonably attainable. Quality is so much more important a factor in electroplating that speed is almost invariably sacrificed if required to produce a good grade of electrodeposit. In actual practice, it is well known to those skilled in the electroplating art that it requires the highest degree of skill, and unremitting care and attention in order to produce consistently good high-grade electrodeposits.

Commercially acceptable electroplating requires a homogeneous uniformly thick and smooth plate. In many cases the plate must be as bright as possible to avoid excessive subsequent buffing and polishing treatment. Industry often accepts relatively non-uniform and unattractively rough, unhomogeneous plating because it either is too costly to secure better work, or, as is often the case, better plating cannot be produced. Mechanical buffing is then relied upon to bring the plated metal to a better condition.

Usually electroplating must be conducted at relatively low current densities in order to be sure to secure a satisfactory metal deposit. Likewise the electrodeposition of metal requires a considerable amount of skill as developed by experience in order to satisfactorily electroplate irregularly shaped objects as by proper disposition of anodes, selecting proper current densities and electrolyte composition. For instance, a cylindrical member such as a tube or a wire can be electroplated at relatively high current densities with the electroplated metal usually being of a fairly high quality. As more and more irregular shapes are subjected to electroplating, many problems begin to present themselves, and it becomes progressively more difficult to secure a uniform and homogeneous electrodeposit. A square sheet is much harder to electroplate successfully than a cylinder while a member having projections, recesses and cavities requires specialized conditions to secure a good plating job.

Particularly great difficulties are encountered in electroplating on base members thick deposits of metal of the order of 10 mils (0.010 inch), thickness and greater. The electrodeposits tend to become progressively more nodular, rough, non-uniform in thickness, and often occur as coarse crystalline or dendritic coatings. It has been recognized that electroplating tends initially to deposit sound metal, but that the deposit becomes disproportionately poorer in structure and smoothness as more and more metal is electrodeposited continuously over the initial deposit.

2

In electroplating a base member from any given solution of electrolyte, the limitation on the current density which may be employed to deposit metal occurs when the electrolyte immediately adjacent the base member becomes depleted of sufficient metal ions to plate out in accordance with the electrical current applied. Thereafter a certain amount of the water in the electrolyte begins to decompose and hydrogen is formed on the surface of the base member. This reduces the plating efficiency. Hydrogen tends to blanket the surface of the base member and thereby greatly diminishes the plating. This phenomenon is known as polarization. Plating is ordinarily conducted at such a rate as to prevent polarization from occurring, at least to a substantial extent. Some polarization appears to occur even in the most carefully conducted plating operations, but ordinarily may be kept within reasonable limits. Polarization causes inefficiency and non-uniformity in plating.

The present invention is directed to the application of a predetermined alternating or reversed current cycle to the base member being plated, the current being so applied that at predetermined intervals a given thickness of metal is electrodeposited on the base member and then reversed so that the given thickness of the electrodeposit is partially depleted whereby unsound and inferior metal is removed. In this manner, the base member is plated so that it acquires a uniform deposit composed of a great number of very thin, homogeneously bonded increments of sound metal. Numerous advantages have been found to follow the electroplating of members by means of the current cycle of this invention.

It has been suggested heretofore, as in Holt Patent 1,534,709, to conduct a plating operation in which at intervals plating is interrupted by briefly reversing the current for a small fraction of a second for the purpose of depolarization only of the plated surfaces and then resuming plating. This procedure has been tried but it does not produce any improvement in the plated metal. By contrast, as disclosed herein by applying a sufficient reverse current for a sufficient period of time to deplate unsound and inferior metal, highly unexpected and desirable results in plating are secured.

The object of this invention is to provide for electrodepositing on a base member a sound and homogeneous electroplate.

A further object of the invention is to electrodeposit on a base member a metal plate by a periodic alternating current process to build up a predetermined electrodeposit from which all unsound and inferior metal has been removed as it tends to be formed.

Another object of the invention is to provide for reversing at periodic intervals the plating cur-

rent applied to a member during the process of plating metal thereon in order to remove unsound or inferior metal, thereby to improve the quality of the plated metal and to impart greater speed and efficiency to the plating operation.

Other objects of the invention will, in part, be obvious and will, in part, appear hereinafter.

For a better understanding of the nature and objects of the invention, reference should be had to the following detailed description and drawing, in which:

Fig. 1 is a view in elevation in section through an electroplating system;

Fig. 2 is a graph plotting time against current employed in the plating cycle;

Fig. 3 is a fragmentary greatly enlarged cross-section through a base member and the electrodeposited thereon by conventional methods;

Fig. 4 is a greatly enlarged fragmentary cross-section of a base member and an electrodeposit produced thereon according to the present invention;

Fig. 5 is a perspective view of an electromagnet; and

Fig. 6 is a perspective through a rectangular frame.

According to my invention, electroplating may be accomplished not only at greater speeds than are ordinarily possible, but more important still, the quality of the electrodeposits produced may be so controlled that they are superior to any attained heretofore in the plating art.

Briefly, it has been discovered that the electroplating process and the electrodeposits produced may be greatly improved by applying to the base member being electroplated an alternating current in which the base member is alternately cathodic for a period of time from about 2 to 40 seconds and is anodic for a period of time from about one-half to 10 seconds, respectively. The anodic phase portion of the current cycle should be of sufficient current density and applied for a sufficient length of time to deplate unsound and inferior metal plated during the preceding cathodic phase portion of the cycle. In particular, the anodic or deplating portion of the cycle should apply at least 10% of the coulombs of current applied to the base member during the cathodic portion of the cycle. For plating nearly all metals, the best results have been obtained where the anodic current phase applies to the base member from 20% to 40% of the coulombs of current applied during the cathodic phase portion of the cycle.

The cathodic portion of the current-plating cycle may be of a current density many times greater than the current density that may be applied to a base member using conventional direct current. Since the plating portion of the cycle only operates from about 2 to 40 seconds, polarization is negligible and it does not build up to as high a degree as would occur if the same current density were employed using direct current. When the current is reversed and the base member is rendered anodic, it frequently is desirable to impart a current density somewhat larger than the plating or cathodic current phase of the cycle. In many cases, excellent results were attained where the anodic current density has been 50% to 100% greater than the cathodic current density.

Many desirable and unexpected results have been obtained by electrodepositing on a base member a metal from an electrolyte using the alternating-current cycle which is the feature of

this invention. The rate of plating to deposit a given thickness of metal on a base member is greatly increased, and in many cases the required thickness of deposit may be applied from the same electrolyte in from 50% to 20% of the time required using only direct current. However, the outstanding advantage is the remarkable quality of the electrodeposited metal produced by the process of this invention. The surfaces of the electrodeposits are much brighter. In many cases, the electrodeposits produced by the practice of the present invention are so highly smooth and polished that nothing comparable has ever been previously secured in any electroplating process. In nearly all cases, with the exception of chromium, as will be explained hereinafter, the smoothness, hardness, uniformity, color, and corrosion-resistance of the metal electrodeposited by the process of this invention are definitely superior to the same metals deposited from the same electrolyte using direct current. Other advantages of the invention will be disclosed hereinafter as the process is described in detail.

Referring to Fig. 1 of the drawing, there is shown an electroplating tank 10 provided with a chemically resistant liner 12 in which is located the electrolyte 14 of a suitable composition to electroplate the desired metal. The conducting bars 16 and 18 are each provided with current from the source 20 of alternating or periodically reversed current meeting the requirements herein set forth. The source of alternating current 20 may be an alternating-current generator designed to generate current according to the desired cycle set forth. In other cases, the source of alternating current 20 may be a direct-current source, such as a battery, generator, or rectifier combined with suitable relays, reversing switches and resistances operated by a timing mechanism to reverse the current at predetermined times in accordance with the requirements of the invention. In other cases, other suitable mechanisms may be devised to produce the desired current cycle. The conductor bar 16 carries a hanger 22 on which there is supported the base member 24 to be electroplated. The hanger 26 supported by the conductor bar 18 carries a suitable anode electrode 28.

By referring to Fig. 2 of the drawing, there is illustrated the alternating-current cycle applied to the member 24 by the current source 20. At the point O—A, the base member 24 becomes cathodic and metal is plated thereon. For most purposes, the current density at A will be higher than that ordinarily employed, everything else being equal, using only direct current. However, it should be understood that it is not necessary to employ greater currents than are normally employed using only direct current. Excellent plating will be secured on the base member even though the current density at A is a value which is less than that normally used. The present invention allows a wider latitude of current densities than previously possible. The only limitation is that the current density at A should not be of such a high value that the electroplated metal is burned or excessive gassing or other undesirable effects occur in the short time that the member is cathodic. The time from A to B may be from about 2 to 40 seconds. The time which is selected will depend on the electrolyte in which the process is being carried out, the shape of the member being plated, and other conditions. The cathodic current from A

to B is shown as a uniform current. However, the current need not necessarily be uniform but may be rippled or pulsating, for example, by superimposing an alternating current on the cathodic direct current, or the current may have a higher value at the point A than at the point B. Ordinarily, however, the current from A to B will be relatively uniform since a uniform current is the most easily and economically secured. At the point B, the current is suddenly reversed to the value C and the member 24 is made anodic. As shown, the anodic current density at C is greater than the cathodic current density. In most cases, it will be found that a higher anodic current density is required to secure the desired results of the invention. However, in many cases, it has been found that the anodic current density may be the same as the cathodic current density. The significant criterion of the anodic or reverse current at C is that it be so correlated to the electrolyte that the plated member be deplated to the extent of removing a substantial amount of plated metal. The anodic current is applied for a period of time of from about one-half to ten seconds based on the corresponding plating or cathodic current. The product of time and the anodic current should have a value in coulombs equal to at least 10%, and preferably 20% to 40%, of the coulombs applied during the cathodic portion of the cycle. The current from C to D need not be uniform as shown, but may be rippled or pulsating or may vary in any predetermined manner. At D, the current is again reversed and the base member is made cathodic and the cycle repeated. In all cases, the cycle will be non-symmetrical. The cycle O—A—B—C—D—E is repeated until suitable thickness of metal has been plated on the base member. The base member is preferably removed from the electrolyte 14 between the portions C and D of the cycle when the member is anodic since the polish of the plated metal is at an optimum at this point.

As the member 24 is subjected to the current cycle shown in Fig. 2, it will be found that metal is plated from the electrolyte 14 at a high rate of speed between the points A and B for from about 2 to 40 seconds. Experience shows that the metal plated during this time is not of a uniform quality but varies. The metal first plated has been found to be of a higher quality and more sound than the subsequent metal, deposited toward the end of the cathodic period, in particular the later plated metal becomes coarser in structure and less dense with an inferior polish and smoothness. Sharp projections, high spots and corners tend to build up plated metal faster than flat areas or recesses. When subjected to the anodic portion of the cycle at point C to D, the unsound and inferior metal is deplated, leaving an electrodeposit of very high quality metal. The deplating portion of the cycle does more than deplate unsound metal. Experience shows that the previously plated metal is preferentially dissolved in such a manner as to remove more metal from the corners, edges and rough projections, such as high spots, nodules, and similar elevated portions from a microscopic standpoint where it was previously plated in excess, than from flat areas and the general surfaces.

Scratches, pores, and other discontinuities and imperfections of the surface of a base member are likewise unusually affected by plating with the alternating current cycle. Referring to Figs. 3

and 4 of drawing, there are illustrated the comparative results between continuous direct current plating and the periodic reverse current plating of this invention, in greatly enlarged cross-sections through a plated base member 30 having a burr 32, a scratch 34, and a pore 36 composed of a relatively non-conducting inclusion, such, for example, as a grain of metal oxide, slag, carbon or sand. On the member of Fig. 3 when subjected to normal direct-current plating, the electrodeposit of metal tends to greatly accelerate its growth at the burr 32 in accordance with well known phenomenon. A nodule 38, accordingly, is produced over the burr 32, particularly if the plating is of any appreciable thickness. At the scratch 34, the electrodeposited metal form an exaggerated valley 40 which comprises relatively sharp ridges thicker than the main portion of the electrodeposited metal and a lesser thickness of metal is deposited in the valley of the scratch than the main portion of the electrodeposited metal. At the pore 36, the electrodeposited metal forms a slightly thicker lip surrounding the pore with substantially no metal deposited over the relatively non-conducting inclusion. It will be apparent that the surface of the plated member 30 in Fig. 3 becomes progressively rougher as plating is carried on. With respect to corrosion resistance, the plated metal is unsatisfactory since there are portions much thinner than the average thickness of the plated metal, and these weaker portions will obviously fail before the main thickness of the plated metal would ordinarily fail.

35 In Fig. 4 of the drawing, there is illustrated the plated base member 30 showing the improvement in electrodeposition accomplished by the practice of my alternating or periodic reverse current plating process. When the base member 30 having a burr 32, scratch 34, and a pore 36 is subjected to plating by the alternating current cycle, there is produced upon the burr 32 a corresponding plated projection with, however, a greater radius and much less difference in height with respect to the main body of the metal adjacent thereto than would occur in direct current plating. No nodules are formed. Over the scratch 34, it will be found that the metal is plated in such a manner as to fill in most of the scratch. 50 Therefore, the scratch is rendered less prominent. Greater protection as well as a smoother surface actually results. The inclusion 36 is soon completely plated over by the process of the present invention. It will be apparent that the surfaces produced by plating according to my invention are smoother than the original base metal surface itself. The uniformity of the plated metal is far superior to any electrodeposit produced heretofore by conventional methods. Of course, it will be understood that only minor or microscopic irregularities are smoothed over. The main contours of the base member are faithfully followed and conformed to by the plated metal.

65 As an explanation of the unexpected results such as are shown in Fig. 4, the following is offered, but I do not wish to be bound strictly to such explanation. Following the plating of metal upon the base member 24 for about 2 to 40 seconds, during the subsequent anodic portion of the cycle unsound and inferior metal is removed and put back into solution immediately adjacent the base member. Any elevations, corners or projections are deplated at a greater rate than the main flat areas of the electrodeposit. Thus

the burr metal 44 deplates more than the rest of the plate. The metal in the scratch 46 is removed at a lesser rate than the lips of the scratch or the plating elsewhere. When the cathodic portion of the plating cycle is again applied to the base member, the metal concentration adjacent the base member is abnormally high, and thereby plating starts and is maintained for part of the period at approximately 100% efficiency in many electrolytes. The metal concentration within and near the scratch 34 is high enough to plate rapidly on both sides of the scratch, and the scratch is filled up from its bottom at a greater rate than the main body of metal is being built up. However, the projections such as 44 do not build up a much greater thickness of metal than does the main body of the plate. Therefore, no nodular or treeing effects are secured. On being repeated, the anodic portion of the cycle again reduces the projections in preference to the scratches or other microscopic depressions and thereby a progressively more uniform surface is secured. It will be apparent that the anodic portion in combination with the cathodic portion of the current cycle imparts new and unexpected characteristics to the plated metal.

Other beneficial effects secured by the anodic portion of the cycle are the replenishing of the metal ions adjacent the base member by deplating inferior and unsound metal. Therefore, the anodic portion of the cycle does not represent wasted energy since plating during the subsequent cathodic portion of the cycle is expedited and is more efficient due to the replenishment of the metal in the closely adjacent electrolyte.

In practicing the invention, exceptionally good results have been obtained in electrodepositing copper, brass, and silver. Electrodeposits of zinc, tin, cadmium, and gold have been produced superior in many respects to those obtained by any conventional plating method. In all these cases, the electrolytes used were those employed in conventional plating practice. No substantial changes in composition are necessary in order to secure the benefits of the present invention. The alternating-current cycle of this invention has been found to give good results not only with conventional plating electrolytes but with electrolytes modified to provide for a better cooperation between the current and the metal being plated. The only exception was encountered in plating chromium; when the reverse or deplating current was applied the base metal deplated instead of the chromium plate.

As examples of various electrolytes and metals that have been plated with the alternating-current cycle of this invention, the following are typical:

#### Example I

An electrolyte was prepared containing:

|                        |                   |      |
|------------------------|-------------------|------|
| Copper                 | ounces per gallon | 7.35 |
| Free potassium cyanide | do                | 1.50 |
| Potassium hydroxide    | do                | 2.48 |
| Addition agent         | ML per gallon     | 8    |

The complex shaped base member 50 shown in Fig. 5 of the drawing was electroplated in a bath as shown in Figure 1. The member 50 is a cobalt ferrous alloy electromagnet having approximately  $\frac{1}{2}$  square foot of surface area. The requirements called for electroplating a thickness of approximately 0.018 to 0.020 inch of copper having a total weight between 28 and 33 grams. It will be readily recognized that plating the member 50 would be quite difficult if a reasonably smooth,

uniform plate were required. The temperature of the electrolyte was varied from 140° F. to 210° F. The pH was maintained at 12 and higher. The electrode 28 was a copper anode. The member 50 was plated in the copper electrolyte according to the following alternating-current cycle:

|         | Time | Current |                         |
|---------|------|---------|-------------------------|
|         |      | Seconds | Ampères per Square Foot |
| Cathode | 15   | 65      |                         |
| Anode   | 3    | 100     |                         |

15 The effective current density was 37 amperes per square foot. In five hours' plating time, several magnets corresponding to member 50 were plated with 31.7 and 32.8 grams of copper, respectively. With the fastest known copper plating system

20 available to the trade using direct-current, the plating of the electromagnets has required from 9 to 11 hours to secure the same weight of copper thereon. Apart from the faster plating by the process of this invention, the copper plate deposited on the member 50 was brighter and smoother than any copper plate heretofore known. It was extremely adherent.

25 Samples of the copper plate produced by the process of this invention were removed from the magnet 50, and the density thereof was found to be approximately 25% to 50% greater than the density of as good a copper plate as could be produced to an equivalent thickness from a direct-current bath of about the same composition. The

30 copper metal produced by the practice of this invention was springy and much harder than conventionally plated copper. The latter, when flexed in the finger, broke readily and had a rough crystalline structure, while the copper

35 plate of this invention when flexed in the hand, did not break but showed considerable elasticity. Upon breaking the copper plate of this invention, the structure was observed to be much finer than the best direct current plated copper.

40 45 Various base members plated with the copper plate using the alternating-current cycle of this invention were far more corrosion-resisting than conventional copper plate. For example, 0.0005 inch of direct-current plated copper on steel

45 50 plates had less corrosion resistance in a salt spray than did 0.00035 inch thickness of copper plate produced by the process of this invention.

#### Example II

55 55 A cyanide copper electrolyte similar to that of Example I was applied to the same member as shown in Fig. 5 of the drawing and electroplated according to the following cycle:

|         | Time | Current |                         |
|---------|------|---------|-------------------------|
|         |      | Seconds | Ampères per Square Foot |
| Cathode | 15   | 90      |                         |
| Anode   | 5    | 90      |                         |

60 The effective current density was 45 amperes per square foot. In 3½ hours 30.37 grams of copper of a thickness of 0.012 inch were deposited on the member. The copper plate was very smooth and shiny in appearance. Electrical tests for the resistance of the copper plate indicated that it was as conducting as 31 grams (thickness 0.018 inch) of copper applied from the same bath over a period of from 11 to 12 hours using direct current.

9

*Example III*

The following Rochelle copper electrolyte was prepared:

|                  | Ounces per gallon |
|------------------|-------------------|
| Copper cyanide   | 4                 |
| Sodium cyanide   | 5.1               |
| Sodium carbonate | 2                 |
| Rochelle salts   | 5                 |

The temperature of the electrolyte was 160° F. 10  
The following alternating-current cycle was applied to the complex surface member of Fig. 5:

|         | Time | Current                 |
|---------|------|-------------------------|
|         |      | Amperes per Square Foot |
| Cathode | 14   | 90                      |
| Anode   | 3.5  | 120                     |

The effective current density was 48 amperes per square foot. The electrodeposit produced was polished and smooth. The copper appeared to be as high a quality as that produced with the straight cyanide electrolyte of Examples I and II.

*Example IV*

An electrolyte for plating brass was prepared as follows:

|                | Grams per liter |
|----------------|-----------------|
| Copper cyanide | 30              |
| Zinc cyanide   | 9.49            |
| Sodium cyanide | 56              |

The temperature of the electrolyte was 100° F. Rectangular steel plates of an area of one-tenth square foot flashed with copper were plated in the brass electrolyte using the following diminishing current conditions:

|         | Time | Current                 |
|---------|------|-------------------------|
|         |      | Amperes per Square Foot |
| Cathode | 3    | 180 to 25               |
| Anode   | 0.8  | 95 to 67                |

The effective current density was 50 amperes per square foot. An unexpected result was that the electrodeposit was a very bright brass. As far as known, it has been desirable to secure a bright brass directly by plating, but this has not hitherto been commercially possible by any known plating process. The tests of the brass plate indicated that it was smoother and more homogeneous than ordinary brass plate as well as being more tenaciously adherent and much more corrosion-resistant. The brass was denser than brass secured by direct current plating.

*Example V*

A zinc-plating electrolyte was prepared with the following constituents:

|                  | Ounces per gallon |
|------------------|-------------------|
| Zinc cyanide     | 8                 |
| Sodium cyanide   | 5                 |
| Sodium hydroxide | 11                |

Rectangular sheets having a surface area of one-tenth square foot were plated in the zinc electrolyte under the following conditions:

|         | Time | Current                 |
|---------|------|-------------------------|
|         |      | Amperes per Square Foot |
| Cathode | 15   | 60                      |
| Anode   | 2    | 65                      |

10

The effective current density was 45 amperes per square foot. A smooth uniform deposit of zinc was produced by the electroplating cycle of this example. The zinc had a surface brightness equal to that produced by the best direct-current processes known at the present time. However, the zinc of this example was deposited as a smoother and more uniform coating than any hitherto produced.

*Example VI*

An electrolyte for plating cadmium had the following composition:

|                | Ounces per gallon |
|----------------|-------------------|
| Cadmium oxide  | 3.5               |
| Sodium cyanide | 14.5              |

A steel member comprising a rectangular sheet of one-tenth square foot area was immersed in the electrolyte and plated with the following current. 20

|         | Time | Current                 |
|---------|------|-------------------------|
|         |      | Amperes per Square Foot |
| Cathode | 15   | 40                      |
| Anode   | 2    | 60                      |

The effective current density was 28 amperes per square foot. The plate of cadmium produced was markedly improved over any direct-current plated cadmium known. The coatings were unusually smooth and had a bright, polished appearance.

In another case, samples of steel were plated in the cadmium electrolyte under the following conditions:

|         | Time | Current                 |
|---------|------|-------------------------|
|         |      | Amperes per Square Foot |
| Cathode | 15   | 60                      |
| Anode   | 2    | 60                      |

The effective current density was 45 amperes per square foot. The cadmium plating secured by following this cycle was of as high a quality as that produced by following the current cycle immediately preceding.

*Example VII*

A silver electrolyte was prepared with the following composition:

|                        | Grams per liter |
|------------------------|-----------------|
| Silver cyanide         | 40              |
| Potassium cyanide      | 62.5            |
| Free potassium cyanide | 40              |
| Potassium carbonate    | 50              |
| Potassium hydroxide    | 10              |

The bath temperature was 80° C. The following alternating-current cycle was employed:

|         | Time | Current                 |
|---------|------|-------------------------|
|         |      | Amperes per Square Foot |
| Cathode | 20   | 11                      |
| Anode   | 4    | 12                      |

<sup>1</sup> Average.

70 The effective current density was 8 amperes per square foot. The silver electrodeposited from this electrolyte using the current cycle indicated was of an extraordinary polished brilliancy. No mechanical buffing or polishing was necessary

75 since it was as bright as could be secured by any

11

mechanical treatment. By comparison ordinary direct-current electroplated silver has an inferior, unattractive and dull appearance. The silver plate produced by the present invention was unusually homogeneous, smooth and uniform. Plated silver using the alternate current of this invention would be completely satisfactory for immediate use. Household silver and any other silver plating that would ordinarily be employed in industry or commerce could be successfully plated by the present process and used without any mechanical buffing or other treatment.

Numerous other plating cycles for plating silver were employed with equally good results. For example, with a cathodic current density of 15 amperes per square foot, the time was varied from 10 to 30 seconds. The anode current densities varied from 50 to 150 amperes per square foot maximum for periods of time from 2½ to 9 seconds. The anodic current densities with silver tended to drop toward the end of the periods. Silver plating may be accomplished using cathode current densities of as high as 100 amperes per square foot.

#### Example VIII

An aqueous solution for plating gold was prepared with essential ingredients as follows:

|                        | Ounces per gallon |
|------------------------|-------------------|
| Gold                   | 0.51              |
| Free potassium cyanide | 0.38              |

The current cycle employed was:

|         | Time    | Current                 |
|---------|---------|-------------------------|
|         | Seconds | Amperes per Square Foot |
| Cathode | 15      | 5                       |
| Anode   | 2       | 10                      |

The effective current density was 3 amperes per square foot. The gold was electroplated upon a rectangular steel base member. The gold was far better both in smoothness and color than any direct-current gold plate known.

The electrolytes of the preceding examples are not exhaustive but are only exemplary of the present invention. In many cases the electrode 28 employed in each of the solutions was of the same metal as that being deposited. However, in plating gold, the electrode was an inert member. The plating can be accomplished satisfactorily according to this invention regardless of the nature of the anodes.

Illustrative of a further advantage of the process of this invention, reference should be had to Fig. 6 of the drawing showing a rectangular open ended casing member 52. The member 52 is a common form of casing for enclosing apparatus and instruments. Hitherto in plating members corresponding to or similar to the member 52, it was necessary to employ an anode inside the frame of member 52 as well as anodes about the exterior of the frame. Even then uneven electroplated deposits often occurred. By using the alternating-current cycle of this invention, it has been found possible to electroplate both the inner and outer surfaces of the frame member 52 quite uniformly without using any internally located anodes or resorting to other time-consuming expedients. The plating of copper on a steel casing corresponding to member 52 resulted in a smooth bright coating over both the interior and exterior surfaces of the member using only

12

external anodes. It was unexpected that the member would be so well plated with only external anodes.

The better distribution of plated metal secured by the alternating-current cycle of this invention as exemplified by the plating of the members of Figs. 5 and 6 constitutes an important feature of the invention. The plating current densities, practicable even with the complex surface members are far higher than would be possible using direct-current plating.

The electrodeposits produced by the invention are superior in both mechanical and chemical properties to plating produced by conventional processes and, therefore, are advantageous for numerous applications requiring the best attainable properties of electroplated metal. Automobile hardware which is subject to abrasion and exposure to moisture and deleterious gases may be advantageously plated with a more durable and corrosion-resistant plating by the process of the present invention. Household appliances subject to heating, food acids, and other corrosive influences will be found to be capable of lasting longer and with better results if produced as herein disclosed. In many cases, particularly in plating copper, silver, and brass electrodeposits, mechanical buffing or polishing may be entirely eliminated since the plated member will be as bright as can be secured by any mechanical polishing operation. Engraving dies, electrotypes, plastic molds and similar members of complex shape may be prepared by electroplating metal base members, graphitic or carbon bodies, wax or resin master patterns dusted with a conducting surface coating of metal powder or graphite in accordance with the present invention to produce a much more durable and wear-resisting plating than can be secured by any known process of plating. The plated metal will be found to be much harder and more corrosion-resistant to conditions encountered in service than ordinary plated metal. The pattern will be followed faithfully without excessive plating on corners and projections. Accordingly, longer wearing dies and printing plates will be attained.

All plating operations regardless of the shape, size or use of the member being plated should be benefited by being conducted with alternating or periodic reverse current in accordance with the teachings of the present invention.

The alternating current plating of the present invention may be carried out in any type of system or apparatus commonly employed for plating. Rubber-covered steel tanks will generally be found to give good results, though wood, glass, or other materials may be employed. The work may be hung on a stationary holder or on a moving conveyor. The size of the apparatus has not introduced any difficulties. Plating with the alternating-current cycle has been carried out as effectively in small glass beakers as well as in large tanks having a capacity of several hundred gallons of electrolyte.

It will be appreciated that alloys as well as single metals may be electrodeposited by the present alternating current process. Several successive deposits of metal in any desirable proportions may be plated on a single member.

The electrolyte may be agitated or distributed in accordance with well known practices in plating. It has been found desirable to maintain a clean electrolyte, for example, by filtering or the like, since the electrodeposits have such a highly polished surface that any solid impurities

from the electrolyte deposited on the plated work are much more apparent than in ordinary electroplating. The temperature of the electrolyte may be varied to suit the plating requirements. The current cycle works as well at temperatures of boiling water as at temperatures below room temperature.

It is intended that all matter contained in the above description or in the accompanying drawing shall be taken as illustrative and not in a limiting sense.

I claim as my invention:

1. The process of electroplating metal from the group consisting of copper, brass, silver, zinc, tin, cadmium and gold on a base member from an electroplating electrolyte in which the deposited metal is readily soluble on the passage of electric current when the base member is the anode, comprising the steps of connecting the base member to be plated into an electroplating circuit including the electrolyte, causing electric current to flow in the plating circuit while the base member is in contact with the electrolyte, the electric current flowing in the plating circuit being periodically reversed so as alternately to electroplate metal on and then deplate metal from the base member, the current for plating metal on the base member being caused to flow for a period of time of not over 40 seconds until a layer of metal is deposited when the current is reversed in direction for a period of time of not over 10 seconds to deplate metal from the base member to remove a portion of the layer of plated metal, the deplating current being of a magnitude and applied for a sufficient period of time to deliver at least 10% of the coulombs delivered during the preceding plating period so that a substantial amount of the plated metal is removed, and repeating the cycle of plating and deplating to cooperate in building up on the base member an electrodeposit in small increments to produce a smooth, sound, homogeneous plate.

2. The process of electroplating metal from the group consisting of copper, brass, silver, zinc, tin, cadmium and gold on a base member from an electroplating electrolyte, the plated metal being one that is readily soluble in the electrolyte upon the passage of an electric current when the base member is the anode, comprising the steps of applying the electrolyte to the base member, passing an electric current through the base member and the electrolyte in a direction to make the base member cathodic for a period of time of not over 40 seconds to electroplate metal on the base member, then reversing the direction of flow of the electric current to make the base member anodic for a sufficient period of time to deliver to the base member at least 10 per cent of the coulombs that were delivered during the preceding cathodic time period to deplate metal which would result in an inferior deposit, and continuing to make the base member successively cathodic and anodic until a desired thickness of metal has been electroplated on the base member.

3. The process of electroplating metal from the group consisting of copper, brass, silver, zinc, tin, cadmium and gold on a base member from an electroplating electrolyte in which the electroplated metal is readily soluble on the passage of an electric current making the base member an anode, comprising the steps of causing electric current to flow through the electrolyte to the base member for not less than 2 seconds and not more than 40 seconds in a direction to make the base member a cathode to plate metal on the

base member and then reversing the flow of current for a lesser period of not less than  $\frac{1}{2}$  second and not more than 10 seconds, respectively, to make the base member an anode to partially deplate the metal plated on the base member, the period and density of reverse flow of current being such as to apply to the base member from 20% to 40% of the coulombs that were applied while the base member was a cathode, and repeating the steps of causing electric current to flow in a direction to plate metal and reversing the direction of flow to deplate part of the metal plated until a desired thickness of metal has been plated on the base member.

4. The process of electroplating metal from the group consisting of copper, brass, silver, zinc, tin, cadmium and gold on a base member from an electroplating electrolyte, the plated metal being one that is readily soluble in the electrolyte on the passage of a current making the base member anodic, comprising the steps of applying the electrolyte to the base member, passing an electric current of predetermined density through the base member and the electrolyte in a direction to make the base member cathodic for a period of time of from 2 to 40 seconds to electroplate metal on the base member, then making the base member anodic and applying a higher anodic current density than the immediately preceding cathodic current density for a period of time sufficient to deliver to the base member at least 10% of the coulombs that were delivered during the preceding cathodic period to deplate metal which would result in an inferior deposit, and continuing to make the base member successively cathodic and anodic until a desired thickness of metal has been deposited on the base member.

5. The process of electroplating sound metal from the group consisting of copper, brass, silver, zinc, tin, cadmium and gold from an electroplating electrolyte having the metal dissolved therein upon a base member immersed therein at an increased rate as compared to continuous direct current plating from the same electroplating electrolyte, the plated metal deposited on the base member being one that is readily soluble in the electrolyte upon the passage of a current making the member anodic, comprising the steps of applying to the base member successive cycles of current each cycle composed of a cathodic portion and an anodic portion to deliver to the base member for a period of time of from about 2 to 40 seconds a cathodic plating current at a density substantially higher than can be effectively applied as continuous direct current to plate the same metal thereon, and then to deliver to the base member an anodic current of a sufficient current density and for a sufficient period of time to deliver to the base member at least 10 per cent of the coulombs delivered during the preceding cathodic portion of the cycle to remove metal plated during the preceding cathodic period which would result in an inferior electroplate, whereby the plated metal is rendered brighter and more homogeneous and has a smoother surface than is obtainable by means of continuous direct current at said cathodic current density from the same electrolyte.

6. The process of electroplating metal from the group consisting of copper, brass, silver, zinc, tin, cadmium and gold on a base member from an electroplating electrolyte, the deposited metal being one that is readily soluble in the electrolyte on the passage of a current making the base member anodic, comprising the steps of apply-

ing the electrolyte to the base member, passing an electric current through the base member and the electrolyte to make the base member cathodic to apply a given cathodic current density thereto for a period of time of from 2 to 40 seconds to electroplate metal on the base member, then making the base member anodic for a time period which is about one-quarter the preceding cathodic period to apply an anodic current at a sufficient current density to deliver to the base member during said anodic period from about 20 to 40 per cent of the coulombs that were delivered during the preceding cathodic period to deplate metal which would result in an inferior deposit, and continuing to make the member successively cathodic and anodic until a desired thickness of metal has been plated on the base member.

7. In the method of electroplating metal from the group consisting of copper, brass, silver, zinc, tin, cadmium and gold on a base member from an electroplating electrolyte in which the plated metal deposited on the base member is readily soluble on the passage of a current when the base member is the anode, the steps comprising passing a plating electric current through the base member while it is in contact with the electrolyte, the plating current being applied for a period of time not less than 2 seconds and not more than 40 seconds to electroplate an increment of the metal, then applying a deplating electric current to the base member to deplate a substantial portion of the preceding increment, the deplating current being of a magnitude and applied for a sufficient period of time to deliver at least 10% of the coulombs delivered during the preceding plating period to effect removal of a part of the previously plated increment, and continuing the alternate plating and deplating until a desired thickness of metal has been applied to the base member.

8. In the method of electroplating a metal from the group consisting of copper, brass, silver, zinc, tin, cadmium and gold on a base member from an aqueous electroplating electrolyte having the metal to be plated dissolved therein and in which the base member is immersed, the steps comprising applying a plating electric current to the base member for not less than 2 seconds and not more than 40 seconds to electroplate an increment of the metal, then applying a deplating electric current for a period of from  $\frac{1}{2}$  to 10 seconds to the base member to deplate a substantial portion of the preceding increment, the deplating current being of a magnitude and applied for a sufficient period of time to deliver at least 10% of the coulombs delivered during the preceding plating period to effect removal of a part of the previously plated increment, and continuing the alternate plating and deplating until a desired thickness of metal is applied to the base member.

9. In the method of electroplating a metal from the group consisting of copper, brass, silver, zinc, tin, cadmium and gold on a base member from an aqueous cyanide electroplating electrolyte hav-

ing the metal to be plated dissolved therein and in which the base member and an anode of the metal to be plated are immersed, the steps comprising applying a plating electric current to the base member for not less than 2 seconds and not more than 40 seconds to electroplate an increment of the metal, then applying a deplating electric current for a period of from  $\frac{1}{2}$  to 10 seconds to the base member to deplate a substantial portion of the preceding increment, the deplating current being of a magnitude and applied for a sufficient period of time to deliver at least 10% of the coulombs delivered during the preceding plating period to effect removal of a part of the previously plated increment, and continuing the alternate plating and deplating until a desired thickness of metal is applied to the base member.

10. In the method of electroplating a metal from the group consisting of copper, silver, zinc, cadmium, and gold on a base member from an aqueous electroplating electrolyte having the metal to be plated dissolved therein and in which the base member is immersed, the steps comprising applying a plating electric current to the base member for not less than about 3 seconds and not more than about 30 seconds to electroplate an increment of the metal, then applying a deplating electric current for a period of from about  $\frac{1}{2}$  second to about 3 seconds to the base member to deplate a substantial portion of the preceding increment, the deplating current being of a magnitude and applied for a sufficient period of time to deliver at least 10% of the coulombs delivered during the preceding plating period to effect removal of a part of the previously plated increment, and continuing alternate plating and deplating until a desired thickness of metal is applied to the base member.

GEORGE W. JERNSTEDT.

#### REFERENCES CITED

The following references are of record in the file of this patent:

#### UNITED STATES PATENTS

| Number       | Name          | Date          |
|--------------|---------------|---------------|
| 1,215,354    | Eaton         | Feb. 13, 1917 |
| 1,534,709    | Holt          | Apr. 21, 1925 |
| 50 1,544,451 | Hambuechen    | June 30, 1925 |
| 1,565,216    | Smith         | Dec. 8, 1925  |
| 1,918,605    | Jones         | July 18, 1933 |
| 2,048,578    | Van der Horst | July 21, 1936 |
| 2,412,698    | Van der Horst | Dec. 17, 1946 |

#### OTHER REFERENCES

Transactions Electrochemical Society, preprint 81-20, Apr. 20, 1942, pages 312-315.

Electroplating, Freeman and Hoppe, 1930, page 100-102.

60 Principles of Electroplating and Electroforming, Blum and Hogaboom, 2d edition, 1930, pages 89, 90, 108, 109, 215-217.